

## UNITED STATES PATENT OFFICE

2,096,390

## COMPOUNDED LUBRICANTS

Arthur W. Burwell, Niagara Falls, N. Y., and Adolf Kempe, Hackensack, N. J., assignors to Alex Corporation, a corporation of New York

No Drawing. Application December 27, 1934,  
Serial No. 759,432

## 5 Claims.

(Cl. 87—9)

This invention relates to the production of lubricating compositions consisting essentially of lubricating oils (usually, lubricating oils of mineral origin) containing dissolved therein substances having the function of imparting to the resulting solutions lubricating properties not possessed by said lubricating oils per se.

In U. S. Patent No. 1,863,004, issued June 14, 1932, to Arthur W. Burwell, there were described the surface tension-reducing effect and improved lubricating effect obtained by adding to a known lubricating oil of mineral origin an oil-soluble addition material obtained by oxidizing a mixture consisting essentially of relatively high molecular weight, saturated, aliphatic hydrocarbons of mineral origin, in the liquid phase, at a temperature of from about 100° to about 175° C. and at a superatmospheric pressure not greater than about 320 pounds per square inch, in the presence of an exciter of oxidation, until the point of incipient formation of compounds which are insoluble in petroleum and in the reaction mixture, which mixture comprises saponifiable and unsaponifiable components, separating the saponifiable components from at least the major portion of the unsaponifiable components, treating the separated portion containing said saponifiable components with steam until substantially no more volatile material passes over, and drying the resulting residue.

In the carrying out of the described oxidation process there are produced in admixture both saponifiable and unsaponifiable oxidation products, the saponifiable components thereof being classifiable into free acids and lactones and esters of those acids. The free acids appear to have, for the most part, the structure of saturated aliphatic hydroxy carboxylic acids of relatively large molecular weight (e. g., an average molecular weight of 300—500). The lactones and esters contents of the saponifiable portion of the oxidation reaction mixture appear to be completely neutral products of reaction between molecules of the aforesaid acids by loss of water, or between the aforesaid acids and alcoholic compounds formed by the oxidation, respectively.

The unsaponifiable portion of the oxidation reaction mixture consists largely of oxygen-compounds of alcoholic, ketonic, and keto-alcoholic constitutions and properties, with or without some unoxidized hydrocarbons.

It has now been found that the aforesaid acidic constituents may be converted into neutral esters thereof, and that the resulting neutral esters possess approximately, but generally to a supe-

rior degree, the same properties with respect to reduction in surface tension and improvement of the lubricity of lubricating oils as those possessed by the aforesaid free acids or mixtures comprising free acids.

According to the present invention the free acids content of the oxidation reaction mixture is esterified by one or another of the optional methods following:

(a) Addition of non-volatile alcohols to the acids, and heating at above 100° C.

(b) Treating the acids with volatile alcohols, in the presence of condensing agents, and thereafter washing with alkali.

(c) Heating, alone, at above 100° C.

Among operable esterifying agents we may use methyl alcohol, ethyl alcohol, propyl alcohol, butyl alcohol, isopropyl alcohol, secondary butyl alcohol, glycerine, glycol, ethylene glycol, and, in general, any commercially known, normally liquid, alcohol.

The free acids content of the oxidation reaction mixture may be esterified by heating the acids with an esterifying agent, e. g., a non-volatile alcohol, at a temperature above the boiling point of water. In carrying this conception into practice the acid is admixed with a non-volatile alcohol, such for instance as glycerine, and the mixture thus made is heated at a temperature above the boiling point of water, e. g., at a temperature of, say, 150° C., for several hours. There is practically no volatilization by this procedure (beyond separation of water), it being found that lower molecular weight acids which may be present readily combine with the high boiling alcohol to form esters.

In accordance with method (b) above, a volatile alcohol, e. g., methyl alcohol, and a condensing agent, e. g., sulphuric acid, are reacted with the acids, the mixture being maintained at a temperature sufficient to keep the mass liquid, or at the temperature, or more or less below the temperature, at which the alcohol boils.

The resulting esterified product may, in any case, finally be treated with an acid-binding agent, such as dilute aqueous alkali (i. e., a solution of not to exceed 1% caustic soda, in water, or an aqueous solution of sodium carbonate of like strength), and then washed with water, to remove any traces of free acid which might not have yielded to esterification.

Discussing the last mentioned method of esterification, it has been found that if the whole oxidation reaction mixture, containing contents of free acids and alcohols produced by the oxida-

55 50 55

tion, be subjected to prolonged heating at a temperature above 100° C. there are formed esters of the free acids, by reaction between the same and alcoholic compounds present in the mixture, with splitting off of water, which latter is separated out by vaporization at the temperature maintained. By practicing this procedure, then, there are produced mixtures of wholly neutral oxygen-compounds of the original hydrocarbons in which 5 neutral mixture the compounds of acidic constitution are present in ester form. This procedure, however, is open to the objection that under the conditions of operation lower molecular weight acids tend to be lost by evaporation, from which 10 acids desirable esters could have been formed. Moreover, the degree of neutralization realized by this procedure may, in particular instances, be found to be insufficient.

As has been indicated hereinbefore, the acids 20 from which the neutral ester mixtures of the present invention are prepared are produced by the liquid-phase, controlled oxidation of mixtures of relatively high molecular weight aliphatic hydrocarbons of mineral origin, such, for instance, 25 as petroleum distillates consisting chiefly of relatively high molecular weight hydrocarbons, amorphous wax such as "Sharples wax", other petroleum-type waxes, and the like. The said oxidation may be practiced under employment 30 of such conditions of temperature, pressure, time, etc., as to yield a reaction product in which little or no unoxidized hydrocarbon remains: oxidation in the presence of a suitable accelerator of oxidation at a temperature of about 140° C. and 35 under a superatmospheric pressure of say 200 pounds per square inch for a period of about 10 hours normally will result in a reaction mixture containing no unoxidized (i. e., "original") hydrocarbons. This condition may be ascertained 40 by recourse to a sulphonation test according to which 1 part by weight of reaction mixture is heated with 3 parts by weight of sulphuric acid for about 30 minutes at a temperature of about 150° C. The absence of unoxidized hydrocarbons 45 in the so-sulphonated mixture is determined by measuring the solubility of the latter in water: if all of the original hydrocarbons have been oxidized the total sulphonation mass will be found to be soluble in water.

50 In a reaction mixture showing by the sulphonation test no unoxidized hydrocarbons there have been found by analysis the following types of compounds: free acids, lactones; alcohols—frequently, poly-alcohols containing from 1 to 3 hydroxyl groups to the molecule; alcohol ketones, in which one of the hydroxyl groups has been further oxidized to the carbonyl group; carbonyl compounds containing no hydroxyl groups and 55 which may contain a plurality of carbonyl radicals; and difficultly saponifiable esters which we shall, in this description, identify as "self-formed" esters.

This invention is predicated upon what is believed to be a new conception of lubrication, 60 namely, that the normally given characteristics of a particular so-called "lubricating oil" (e. g., specific gravity, fire, flash, viscosity, color, etc.) do not necessarily foretell whether or not that 65 particular oil is operable in a given relation, and that in most instances an oil must be "constructed" in the light of the requirements of the intended particular application thereof. While the 70 above-mentioned characteristics are important to the refiner (in order that he may be able to

reproduce a given refined oil) they have little if any bearing on the actual lubricating properties of the oil. Thus, it has been found that the viscosity of an oil is not, in general, an index of its relative resistance to film rupture. Resistance 5 to film rupture is more dependent upon the individual "oiliness" of the oil than upon its viscosity: oils of the highest viscosity at high temperature may show easy film rupture at low pressure and at low temperature. On the other 10 hand, it is possible to construct oily lubricating compositions of low relative viscosity which compositions show high resistance to film rupture under the most exacting conditions of pressure 15 and temperature.

A probable explanation is that the film which constitutes the actual lubricating material between the surfaces to be lubricated is not closely related to the oil as a whole: it is related only to the mixture of bodies which are segregated 20 at the surfaces and which form the actual lubricating film. If there are present in the oily composition bodies which will be segregated at the surfaces and which are capable of resisting film rupture to a determined high point of pressure 25 and temperature, then that oily composition will, regardless of its actual Saybolt viscosity, function properly within the ranges specified and at all temperatures, and pressures, below those shown as the final ones at which the film shows rupture.

Exhaustive tests of oily lubricating compositions, over wide ranges of pressures and of temperatures, have demonstrated the unforeseeable fact that the addition to "straight" petroleum lubricating oils of one or more non-acidic oxidized petroleum hydrocarbons materially improves the "oiliness" of the oils, enabling films thereof to withstand rupture at higher pressures and/or temperatures than a film of the "straight" oil could withstand, while generally simultaneously reducing the drag, or internal friction, of the oil film at all pressures. These tests were made in several ways: in one way the oil was maintained at, say, 212° F. and tested at all pressures from zero to 1500 or 2000 pounds. In a 45 second mode of examination, the pressure was held at, say, 1500, or 2000, pounds, and the oil was tested at all temperatures between, say, 140° F. and 400° F. (this latter range covering all temperatures normally encountered in the crank-case, on the wrist pins, and even on the upper rings of the pistons of an automobile engine). It was found, through the carrying out of these tests, that it is possible to construct, from almost any "straight" petroleum lubricating oil—regardless of actual Saybolt viscosity—oily lubricating compositions having almost any predetermined desired film strength and/or desired low coefficient of friction by proper incorporation into the "straight" oil of relatively small but effective amounts of the hereinbefore discussed non-acidic oxidized petroleum hydrocarbons.

The invention will be described in further detail by reference to the following illustrative specific examples:

1.—Into a still or other closed vessel equipped with means for heating the contents thereof were charged 1 pound of acids derived from the oxidation of amorphous wax (i. e., "Sharples" wax), derived from petroleum oil, and .06 pound of 70 glycerine. The mixture of acids and glycerine was brought up to a temperature of 110° C. within twenty minutes and maintained at about that temperature for eighty-six hours. The acids and glycerine reacted to form the glycerol esters of 75

the acids, water being evolved and distilled off. During the treatment a stream of an inert gas was passed through the reaction mixture, to agitate the latter and to carry off water vapor as formed. The resulting esterified product was approximately neutral, only 1.4 cc. of normal alkali solution being required to neutralize the free acid content of a 10 gram sample of said product. The original acidity for 10 grams was 10 16.2 cc.

## KOH

n

One part of the so-produced esterified product was admixed with 199 parts of a motor lubricating oil. The resulting composition was found to have a much lower coefficient of friction, and lower tangent friction drag, at bearing loads of from 500 to 1000 pounds per square inch, than did the same oil without the ester addition.

2.—A portion of the esterified product of Example 1 was washed with a 1% aqueous solution of caustic soda until by test it showed no free acid.

The washed esterified product was blended with motor lubricating oil in the proportion of 0.75 part of the esterified material to 99.25 parts of the oil. The resulting composition was found to have an improved "lubricity" over that of the oil per se, as evidenced in lowered coefficient of friction and in lowered tangent friction drag.

3.—150 pounds of sulphuric acid, oil vitriol, were added slowly to 400 pounds of methanol, under agitation, and the mixture was cooled. 100 pounds of methanol were added to 400 pounds of the acidic saponifiable material derived from the oxidation of amorphous wax (i. e., "Sharples" wax), and this mixture was heated, under agitation and reflux, to 60° to 65° C. While this temperature was maintained the cooled mixture of methanol and sulphuric acid was added to the heated mixture slowly (over a period of from 1 to 2 hours' time), and the reaction mixture was heated and agitated, under reflux, at 60-65° C. until by test it was determined that a maximum of esterification had been reached. The reaction mixture was then admixed with water, whereby to dissolve the catalyst (i. e., the sulphuric acid), the ester mixture was separated from the aqueous solution of sulphuric acid, and the separated ester mixture was washed with water and then with dilute aqueous sodium carbonate solution (1%) to remove any unesterified acids.

The resulting methyl ester mixture was found to improve the lubricity of a lubricating oil. In this connection it may be mentioned that the smaller the molecule of the alcohol used in esterifying the acid the more pronounced appears to be its lubricity-improving properties. It may be remarked that there appears to be a direct ratio between the amount of oxygen (relative) in the compound and the degree of lubricity-improving effect produced by that compound.

4.—The procedure of Example 3 has been carried out using another relatively low molecular weight alcohol in place of the methanol: thus, ethanol, propanol and other similar alcohols have been found to be operable in the production of neutral esters of the aforesaid acids, which esters were found to have desirable lubricity-increasing properties.

Other catalytic assistants of esterification may be used in place of the sulphuric acid of Example 75 3, e. g., another inorganic acid. Zinc chloride,

and calcium chloride, have been found to be operable assistants also.

The ester mixtures so formed have, in general, physical properties similar to those of the non-esterified products: they differ therefrom in having lower melting points, a more pleasant odor, and greater solubilities in petroleum hydrocarbons.

We have discovered, also, that the hereinbefore described esterification of the free acids contents of oxidation reaction mixtures prepared as above described may be effected without having recourse to separation of the acids from other, co-existent, oxidation products. Thus, we have found that the acids content of the hereinbefore described "saponifiable" portion of the crude oxidation reaction mixture may be converted into neutral esters by practicing the above described esterification procedure upon the "saponifiables" separated from said crude oxidation reaction mixture, and that the resulting neutral mixtures have lubricity-improving properties similar to those of the isolated synthesized esters. In carrying out this embodiment of the invention we determine the content of free acids in the "saponifiable" portion and react the said portion with alcohol (in accordance with the procedure of Examples 1, 2 and 3 above) in that amount which is calculated to be necessary for maximum esterification of that free acids content. When maximum esterification has been effected the catalyst (if any catalyst has been used) is removed, and any residual free acid, if there be any, may be separated out by cautious treatment of the product with a dilute aqueous solution of soda ash or caustic soda and washing with water. The resulting mixture, consisting essentially of esterized acids, self-formed lactones and esters, is a neutral lubricant aid which readily dissolves in lubricating oil and which when added to lubricating oil serves

30  
35  
40  
45  
50  
55  
60  
65  
70  
75

to increase the lubricity of the latter.

The free acid-containing oxidation reaction mixture (derived from a petroleum hydrocarbon mixture by practicing thereon the hereinbefore described oxidation procedure) as a whole may be heated at a temperature above the boiling point of water for some hours, water being driven off, whereby to produce the maximum amount of lactones and self-formed esters in said mixture, any residual free acid therein thereafter being either (1) neutralized and removed or (2) esterified by means of alcohol (preferably, a low molecular-weight alcohol such as methanol or ethanol). The resulting neutral or substantially neutral mixtures are of high value as lubrication addition materials.

Lastly, the whole (i. e., crude) oxidation reaction mixture, containing a content of free acids, may be treated by ascertaining the amount of free acids contained therein and esterifying those free acids with added alcohol (either with a high molecular-weight alcohol, at a temperature above 100° C., or with a low molecular-weight alcohol with the aid of a condensing agent, at a temperature below 100° C.), any residual (i. e., un-esterified) acid then being removed, yielding a mixture of wholly neutral compounds which mixture has lubricity-improving properties. It is to be noted that this last-mentioned mixture differs from that produced by (1) prolonged heating of the crude oxidation reaction mixture followed by (2) esterification of residual free acid in that the latter product contains a relatively larger proportion of lactones than the former, and in that

the esters of the latter product are not identical with the esters of the former.

When unesterized acid mixtures are attempted to be dissolved in petroleum (e. g., in lubricating oil of petroleum origin) there is normally a tendency for the relatively low molecular weight, highly oxygenated acids to drop out of solution. However, the esterized acids are characterized by the common property of being easily soluble in petroleum. Esterization, therefore, is of value for the reason that it makes possible the retention and use of these less readily soluble acids in lubricating compositions. It is probably for this reason, also, that the esterized acids are more valuable as lubricity-increasing agents than are the acids not so esterized. Higher film strengths and lower coefficients of friction are attained by use of the esterized acids than are attained by the use of the corresponding free acids.

4.—1 pound of the saponifiable portion of a crude oxidation reaction mixture obtained, by the oxidation procedure hereinbefore described, from a 36°-40° distillate of Pennsylvania petroleum, which saponifiable portion upon analysis showed a free acids content of 30% by weight, were admixed with 0.1 pound of glycerine, this being a large excess of glycerine, and the mixture was heated in a still to about 150° C., while agitating the mixture and removing evolved water therefrom by blowing a stream of a non-reactive gas therethrough. The heating was continued at about 150° C. for thirty-one hours. The resulting product was found to contain a residual acid (free acid) content equivalent to 1.3 cc. of normal alkali per 10 gram sample of the esterized product, which free acid content was too immaterial to warrant removal as by treatment with very dilute alkali solution.

We have found that while the amount of the neutral esters, or of the esterized "saponifiables" portion of the oxidation reaction mixture, to be added to the lubricating oil may be varied, and while the determination of the amount to be added depends upon a number of factors including especially the intended use of the resulting lubricating composition, the characteristics of the oil used, etc., it may be stated that the amount to be added to a lubricating oil intended for use in the crankcase of an automotive engine will range from 0.25% by weight up to, say, 0.75%. In the case of cylinder oils, we may use from 1 to 2% of the esterized material. The use of larger proportions of the esterized material, e. g., up to about 4 to 6%, with lubricating oils affords very tough films (of lubricant) under wide ranges of pressure. The addition of these esterized materials to the constituents of greases has proved valuable for two reasons: (1) they greatly reduce the high drag of the grease and (2) they make possible the easy solution in the grease of highly chlorinated aromatic hydrocarbons (e. g., high chlorinated naphthalenes) widely used in high pressure greases. Thus, for example, we have found that a pressure grease having very desirable properties may be prepared from a 750 fire test cylinder stock of Pennsylvania origin, having a viscosity of about 400-450 at 210° F., plus 8%

of highly chlorinated naphthalene plus 4-6% of esterized product derived from the oxidation products of amorphous wax and paraffin in about equal proportions.

While in the foregoing the invention has been described with reference to synthetic esters produced by reacting aliphatic alcohols with free saturated aliphatic hydroxy carboxylic acids of high molecular weight, said acids being obtained, in association with other saponifiable bodies and with unsaponifiable oxygenated bodies, by the controlled, liquid-phase, partial oxidation of hydrocarbon mixtures of mineral origin at a temperature between about 100° C. and about 175° C. and at a superatmospheric pressure not above about 320 pounds per square inch, in the presence of an exciter of oxidation, the invention is not restricted thereto but consists broadly in the provision of a lubricating composition consisting essentially of a solution, in hydrocarbon lubricating oil, of a relatively small amount of a synthetically prepared, neutral, ester.

This application contains subject matter in common with our application Serial No. 700,018, filed November 27, 1933.

25

We claim:

1. A lubricating composition consisting of a major amount of lubricating oil of mineral origin and dissolved therein a minor amount of neutral aliphatic alcohol esters of the free saturated aliphatic hydroxy carboxylic acids content of an oxidation reaction mixture obtained by the controlled liquid-phase oxidation of hydrocarbons of mineral origin at a temperature between about 100° C. and about 175° C. and at a superatmospheric pressure not above about 320 pounds per square inch, in the presence of an exciter of oxidation, the alcohols being members of the group consisting of relatively low molecular weight, normally liquid, aliphatic alcohols including glycerin and glycol, and the alcohols derived from the aforesaid mineral hydrocarbons in the production of the aforesaid acids.

2. A lubricating composition as defined in claim 1, in which the alcohol is methyl alcohol.

3. A lubricating composition as defined in claim 1, in which the alcohol is glycerin.

4. A lubricating composition as defined in claim 1, in which the alcohol is one derived from said mineral hydrocarbons in the production of said acids.

5. A lubricating composition consisting of a major amount of lubricating oil of mineral origin and dissolved therein a minor amount of neutral low molecular weight aliphatic alcohol esters of the free saturated aliphatic hydroxy carboxylic acids content of an oxidation reaction mixture obtained by the controlled liquid-phase oxidation of a hydrocarbon mixture of mineral origin at a temperature between about 100° C. and about 175° C., and at a superatmospheric pressure not above about 320 pounds per square inch, in the presence of an exciter of oxidation.

ARTHUR W. BURWELL. 65  
ADOLF KEMPE.